

## UNITED STATES PATENT OFFICE

2,588,280

## LUBRICATING GREASE

Rosemary O'Halloran, Elizabeth, and John J. Kolfenbach, Somerville, N. J., assignors to Standard Oil Development Company, a corporation of Delaware

No Drawing. Application August 26, 1949,  
Serial No. 112,644

7 Claims. (Cl. 252—40)

1

This invention relates to a lubricating grease composition which has improved structural stability due to the presence of a selected range of fatty acid constituents.

Recent developments in grease technology have indicated an increasing need for greases of smooth structure which will provide satisfactory lubrication over a wide range of temperature conditions. It is desirable that such greases should also possess water resistance properties and high dropping points. It is widely recognized that these properties are to be found in mixed base greases, for example soda-barium greases, and in lithium greases. These greases are customarily prepared from their respective soaps of saturated fatty acid mixtures. Lithium and sodium-barium soaps can be dispersed in high V. I. oils and are therefore suitable as thickening agents in greases required to operate under widely varying temperature conditions, which is of special interest in the aeronautical field. In general, soaps are more difficult to disperse in high V. I. oils and greases employing high V. I. oils are subject to loss of structure upon extended working.

It is an object of this invention to provide a lubricating grease composition which is satisfactory for the lubrication of metal surfaces over a wide range of temperature conditions, and which has superior structural stability toward mechanical working.

It has now been found that the molecular weight distribution of the fatty acids employed in making these greases has a marked influence on their structural stability. This invention, therefore, comprises a lubricating grease composition which employs as the soap constituent a metal salt or a mixture of metal salts of substantially saturated fatty acids, the composition of the acid mixture being controlled so as to have a preferred molecular weight distribution.

For manufacturing grease compositions having the optimum structural stability, the mixture of fatty acids employed should contain 50% or more by weight of a single substantially saturated aliphatic acid having a carbon chain length within a range of from 16 to 22 carbon atoms and about 10% to about 30% by weight of a single saturated aliphatic acid having a carbon chain length 4 carbons fewer than the major component, that is to say, having a carbon chain length within the range of from 12 to 18 carbon atoms. The mixture of acids can, of course, have a certain amount of acids other than the two principal acids just described.

2

It is to be recognized, that the description of the fatty acids may be varied. For instance, since the molecular weight varies directly with the chain length, the preferred distributions may be expressed in terms of molecular weight ranges. In using this terminology the mixture of acids employed may be described as containing 50% or more of a substantially saturated aliphatic acid having a molecular weight range of 256 to 340 and from about 10% to 30% by weight of a substantially saturated aliphatic acid having a molecular weight within a range of 200 to 284.

The optimum combination of acids necessary to achieve structural stability may be arrived at by proper combination of commercially available fatty acids of well defined molecular weight distribution. For this application the various hydrogenated fish oil acids are not well suited. The molecular weight spread of the fatty acids in these mixtures vary markedly, since these acids represent distilled cuts of mixtures of acids containing variable amounts of  $C_{12}$  to  $C_{22}$  acids. The hydrogenated tallow acids, however, represent a fixed distribution, containing only  $C_{16}$  and  $C_{18}$  in essentially constant ratio. Employing a major proportion of an acid of fixed molecular weight distribution and a smaller proportion of an acid to provide the desirable distribution ensures more reproducible distribution. In the cases cited below, this was accomplished by the use of commercial myristic acid or hydrogenated sperm oil acids, which consist principally of myristic and lauric acids. It will be obvious that many other combinations are possible, such as a mixture containing 50 to 90% of pure palmitic acid, and 10 to 30% of lauric acid. Another example is behenic acid which is prepared by hydrogenating rape oil acids, and therefore contains about 85 to 90% behenic acid, and 10 to 15% stearic acid. However, the use of pure fatty acids to obtain the desired mixture is prohibitively expensive, so that the combination of hydrogenated tallow acids and hydrogenated sperm oil acids is to be preferred. These acids possess the narrowest molecular weight range of available commercial acid mixtures. This mixture of acids is actually somewhat less expensive than the special fractionated hydrogenated fish oil acids. By the use of this acid mixture the molecular weight distribution of the total mixture is fixed, since in the preparation of the mixture, approximately 72% of acids of a definite molecular weight range distribution are employed.

As an example of the application of this invention, and not to limit it in any way, several greases of the soda-barium (mol ratio 17/1) type were prepared according to the following general formula and method of manufacture.

## EXAMPLE I

15.0% Fatty acids (saturated)  
 2.0% NaOH  
 0.9% Ba(OH)<sub>2</sub>·8H<sub>2</sub>O  
 12.4% Phenol extracted coastal distillate, 37  
 SUS/210° F. viscosity  
 0.4% Phenyl-alpha-naphthylamine  
 69.3% Phenol extracted Panhandle distillate, 44  
 SUS/210° F. viscosity

The barium hydroxide was added (10% in water) to a mixture of the fatty acids and the coastal distillate at 150° F. The mixture was stirred for 15 minutes. The sodium hydroxide (30% in water) was then added, and the mixture was dehydrated. The Panhandle distillate was added, the mixture heated to 400° F. and a sample taken for free acidity. The free acidity (A. S. T. M. D128-47 Method) was adjusted to 0.4% as oleic acid, the phenyl alpha naphthylamine was added and the grease was panned in 5-inch layer. After cooling for 10-16 hours, the grease cake was transferred to the A. S. T. M. motorized grease worker and the penetration after 60,000 strokes with the fine hole worker plate was determined as a measure of structure stability (345-350 mm./10, A. S. T. M. penetration on the cooled grease after an additional 60 strokes with the coarse hole plate being considered borderline).

The molecular weight distribution of the acids employed was varied either by selecting commercial acids of determined distribution, or by mixing acids of known molecular weight distribution. The acids employed, the molecular weight distribution in terms of number of carbons in the acid, and the stability of the greases to mechanical working are shown in Table I.

TABLE I  
*Effect of molecular weight distribution on structural stability*  
 [Na/Ba Grease Containing 16% Soap in Mineral Oil Base Stock<sup>1</sup>]

| Mixture                                                                           | Molecular Weight Distribution |                 |                 |                 |                 |                 | Penetration, mm./10 60,000<br>× Fine Hole Plate <sup>2</sup> |
|-----------------------------------------------------------------------------------|-------------------------------|-----------------|-----------------|-----------------|-----------------|-----------------|--------------------------------------------------------------|
|                                                                                   | C <sub>12</sub>               | C <sub>14</sub> | C <sub>16</sub> | C <sub>18</sub> | C <sub>20</sub> | C <sub>22</sub> |                                                              |
| Ex. 1 Myristic Acid <sup>3</sup>                                                  | 6.1                           | 89.7            | 3.7             | —               | —               | —               | Does not disperse in oil.                                    |
| Ex. 2 Hydrofol 30 Acids <sup>4</sup>                                              | 24.9                          | 37.6            | 30.6            | 3.4             | —               | —               | Do.                                                          |
| Ex. 3 Hydrofol Acids 51 HO <sup>5</sup>                                           | —                             | 15.8            | 56.6            | 20.4            | 3.4             | 1.2             | 350 (Marginal).                                              |
| Ex. 4 Hydrofol Acids 405 <sup>5</sup>                                             | —                             | 1.2             | 20.4            | 76.8            | —               | —               | 348 (Marginal).                                              |
| Ex. 5 Stearic Acid <sup>3</sup>                                                   | —                             | —               | 55.0            | 45.0            | —               | —               | 361 (Unsatisfactory).                                        |
| Ex. 6 Hydrofol Acids 53 <sup>5</sup>                                              | —                             | 7.3             | 31.0            | 23.7            | 21.8            | 12.0            | 365 (Unsatisfactory).                                        |
| Ex. 7 Hydrofol Acids A.B. <sup>5</sup>                                            | —                             | 1.7             | 13.3            | 16.9            | 37.4            | 28.4            | 370 (Unsatisfactory).                                        |
| Ex. 8 50% Hydrofol Acids 405 <sup>6</sup><br>50% Myristic Acid <sup>3</sup>       | 3.0                           | 45.6            | 12.2            | 38.4            | —               | —               | Fluid (Unsatisfactory).                                      |
| Ex. 9 Behenic Acid <sup>3</sup>                                                   | —                             | —               | —               | 11.7            | —               | 87.0            | 310 (Satisfactory).                                          |
| Ex. 10 90% Hydrofol Acids 405 <sup>6</sup><br>+10% Myristic Acid <sup>3</sup>     | 0.6                           | 10.1            | 18.7            | 69.0            | —               | —               | 305.                                                         |
| Ex. 11 70% Hydrofol Acids 405 <sup>6</sup><br>+30% Myristic Acid <sup>3</sup>     | 1.8                           | 27.8            | 15.4            | 53.6            | —               | —               | 334.                                                         |
| Ex. 12 70% Hydrofol Acids 405 <sup>6</sup><br>+30% Hydrofol 30 Acids <sup>4</sup> | 7.5                           | 12.1            | 23.5            | 54.8            | —               | —               | 310.                                                         |

<sup>1</sup> Blend of 85% by weight of a phenol extracted Panhandle distillate having a viscosity at 210° F. of 44 S. U. S. and 15% by weight of a phenol extracted coastal distillate having a viscosity at 210° F. of 37 S. U. S. The viscosity index of the blend is 92.

<sup>2</sup> Penetration taken after grease cooled to room temperature and was worked an additional 60 strokes with large hole plate.

<sup>3</sup> Commercial grade.

<sup>4</sup> Hydrogenated sperm oil fatty acids.

<sup>5</sup> Hydrogenated fish oil fatty acids.

<sup>6</sup> Hydrogenated tallow acids.

These data indicate that a high percentage of a single molecular weight acid is desirable providing that the single acid has a carbon chain

length of 16 carbon atoms or above. This is shown by Examples 1 and 2 wherein a high concentration of C<sub>12</sub> and C<sub>14</sub> acids did not produce any grease structure. In addition to the required higher molecular weight portion, however, it is necessary to have a minor amount of lower molecular weight material. Examples 3, 4, and 5 contain appropriate amounts of the desirable higher molecular weight constituents, but lack the lower weight material. A very broad range of molecular weights, illustrated by Examples 6, 7, and 8 are shown to be the least desirable of all. Therefore, for optimum results the fatty acids employed should be concentrated in molecular weight about a single molecular weight species, not less than C<sub>16</sub> and preferably C<sub>18</sub>, but should contain a minor proportion, i. e. from 10% to 30% by weight, of an acid having an average chain length of about 4 carbon atoms fewer than the chain length of the acid present in the largest amount. In other words, the preferred embodiment of this invention contemplates employing a mixture of fatty acids wherein from 50 to 90% by weight of the mixture has an average carbon chain length of from C<sub>16</sub> to C<sub>22</sub>, and from 10 to 30% of an acid having a carbon chain length within a range of from C<sub>14</sub> to C<sub>18</sub>. Examples 9, 10, 11, and 12 illustrate the preferred greases. These greases have a dropping point within the range of 325-340° F.

In addition to the utility of this invention in mixed base soda soap greases, it has also been shown that a controlled mixture of fatty acids will effect an improvement in the shear stability of lithium soap greases. Two greases were prepared according to this general formula and method of manufacture.

## EXAMPLE II

13.9% by weight, Fatty acids (saturated)  
 2.2% by weight, LiOH. H<sub>2</sub>O  
 0.5% by weight, Phenyl alpha naphthylamine  
 83.4% by weight, phenol extracted coastal distillate (Vis. at 210° F./45 SUS)

The acid was mixed with 1/4 of the total amount of the base oil, heated to 150° F. and the lithium hydroxide was added as a boiling water solu-

tion. The mixture was dehydrated, oiled back, and was heated until a temperature of 400° F. was reached. The phenyl alpha naphthylamine was added and the mixture was pan cooled in a 4 inch cake. The free acidity was found to be 0.06%, calculated as oleic acid (A. S. T. M. D128-47 Method).

The first of these lithium greases was made with a commercially available hydrogenated fish oil acid ("Hydrofol 51 HO") which is widely used in lithium soap grease manufacture. The second grease was made from a mixture of acids. The mixture was formulated according to the concept of this invention, and was one of the mixtures which gave optimum results in the case of the soda-barium grease. It had a dropping point in the neighborhood of 380° F. The acids employed, the molecular weight distribution in terms of the number of carbons in the acid, and the stability of the grease to mechanical working are shown in Table II.

important feature of the invention is that the mixture of acids be distributed largely around a single molecular weight with a minor amount of acids of a molecular weight about 56 units less than the molecular weight of the acid present in predominant amount.

What is claimed is:

1. A lubricating grease composition which consists essentially of a lubricating oil thickened to a grease consistency with from 10 to 20% of a mixture of the sodium and barium salts of a mixture of substantially saturated aliphatic acids, said mixture of acids containing from 10 to 90% by weight of an acid in the C<sub>16</sub> to C<sub>22</sub> range and from 10 to 30% by weight of an acid having 4 less carbon atoms than the acid present in the predominant amount.

2. A lubricating grease composition which consists essentially of a lubricating oil thickened to a grease consistency with a mixture of the sodium and barium salts of a mixture of substantially

TABLE II

## Effect of molecular weight distribution on structural stability

[Lithium Grease Containing 15% Soap in Mineral Oil Base Stock<sup>1</sup>]

| Mixture                                                                                    | Molecular Weight Distribution |                 |                 |                 |                 |                 | Penetration, mm/10 100,000<br>x Fine Hole Plate <sup>2</sup> |
|--------------------------------------------------------------------------------------------|-------------------------------|-----------------|-----------------|-----------------|-----------------|-----------------|--------------------------------------------------------------|
|                                                                                            | C <sub>12</sub>               | C <sub>14</sub> | C <sub>16</sub> | C <sub>18</sub> | C <sub>20</sub> | C <sub>22</sub> |                                                              |
| Example 1:<br>Hydrofol Acids 51 HO <sup>3</sup> .....                                      |                               | 15.8            | 56.6            | 20.4            | 3.4             | 1.2             | Semi-fluid.                                                  |
| Example 2:<br>Hydrofol Acids 405 <sup>4</sup><br>+30% Hydrofol 30 Acids <sup>5</sup> ..... | 7.5                           | 12.1            | 23.5            | 54.8            | -----           | -----           | 345.                                                         |

<sup>1</sup> Phenol extracted coastal distillate of 45 SUS/210° F. viscosity and 70 viscosity index.

<sup>2</sup> Penetration taken after grease cooled to room temperature and was worked additional 60 strokes with large hole plate.

<sup>3</sup> Hydrogenated fish oil fatty acids.

<sup>4</sup> Hydrogenated tallow fatty acids.

<sup>5</sup> Hydrogenated sperm oil fatty acids.

These data indicate that a grease formed from the lithium salts of a mixture of acids having controlled molecular weight distribution prepared according to the concept of this invention is of excellent stability.

It will be understood by those familiar with the art that the soap content of greases will vary widely depending upon the consistency desired, the presence of additives and the nature of the lubricating base oil. The examples cited above contain about 15% soap, but this is in no way limiting on the invention, since superior greases can be prepared using from 5 to 50% soap providing the optimum fatty acid molecular weight distribution is maintained.

In summation, this invention comprises the manufacture of improved lubricating grease compositions which have excellent lubricating qualities within a wide range of temperatures and, in addition which are not subject to loss of structural stability under prolonged conditions of shear. The grease compositions are made using salts of alkaline earth metals or alkali metals, or mixtures thereof, of substantially saturated aliphatic acids, said acids containing 50% to 90% of a single acid having from 16 to 22 carbon atoms and from 10% to 30% of another single acid having from 12 to 18 carbon atoms. It is to be understood, of course, that the mixture of acids can contain a certain amount of acids which do not fall in either of these categories. However, the

15 saturated aliphatic acids, said mixture of acids containing from 50 to 75% by weight of a C<sub>18</sub> acid and from 10 to 30% by weight of a C<sub>14</sub> acid.

3. A lubricating grease composition according to claim 1 in which the mixture of acids contains from 15 to 25% by weight of an acid having 16 carbon atoms.

4. A lubricating grease composition according to claim 1 in which the mixture of acids contains from 1 to 10% of an acid having 12 carbon atoms.

5. A lubricating grease composition according to claim 1 in which the mixture of acids contains substantially no acid having more than 18 carbon atoms.

6. A lubricating grease composition according to claim 1 in which the mixture of acids is a commercial behenic acid.

7. An improved lubricating grease composition having a superior structural stability which consists essentially of a mineral base lubricating oil thickened to a grease consistency with the sodium and barium salts of a mixture of substantially saturated fatty acids, said mixture of acids having the following molecular weight distribution:

|                                       | Per cent<br>by weight |
|---------------------------------------|-----------------------|
| C <sub>12</sub> .....                 | 7.5                   |
| C <sub>14</sub> .....                 | 12.1                  |
| C <sub>16</sub> .....                 | 23.5                  |
| C <sub>18</sub> .....                 | 54.8                  |
| 75 Greater than C <sub>18</sub> ..... | 2.1                   |

and containing incorporated therein 0.4% by weight of phenyl alpha naphthylamine.

ROSEMARY O'HALLORAN.  
JOHN J. KOLFENBACH.

## REFERENCES CITED

The following references are of record in the file of this patent:

## UNITED STATES PATENTS

| Number    | Name             | Date          |
|-----------|------------------|---------------|
| 2,229,030 | Adams et al.     | Jan. 21, 1941 |
| 2,229,041 | Brunstrum et al. | Jan. 21, 1941 |
| 2,229,042 | Brunstrum et al. | Jan. 21, 1941 |
| 2,245,702 | Morway           | June 17, 1941 |